

## UNITED STATES PATENT OFFICE

ALBERT HANAK, OF PHILADELPHIA, PENNSYLVANIA

## PROCESS FOR SEPARATING AND RECOVERING OF LEAD FROM TIN OR TIN ALLOYS

No Drawing. Application filed December 15, 1930, Serial No. 502,627. Renewed October 12, 1932.

One object of the invention is to completely separate and recover, primarily, lead, but also other metals, like zinc for instance, from tin, antimony or certain alloys of tin and 5 alloys of antimony. Another object of the invention is to lower the lead content of said metals and alloys to any desired amount and thereby render them industrially more useful. A third object is to purify said metals 10 or alloys by removing any lead and other constituents like zinc, cadmium, etc., which are present as chance impurities only.

Both in the primary or ore smelting, as well as in the secondary non-ferrous smelting industry, there are produced certain 15 metals and alloys which are unsuited for many industrial applications. Thus, if tin or antimony ores contain appreciable amounts of lead, or residues and byproducts 20 containing chiefly tin or antimony or their alloys, become admixed with lead-containing materials, the metals and alloys resulting from the smelting of such material will contain lead and very often this detracts 25 from their value and usefulness. Up to the present time, no simple and economical process was known to remove and recover such lead. The methods which are in general use to purify tin, antimony and their alloys 30 do not remove and recover lead. The electrolytic refining may accomplish the separation of lead from tin or antimony but it requires a great capital outlay to conduct it on a commercial scale and it is otherwise also 35 very costly and involved, especially in case of rather impure metals and alloys. When the lead and other constituents amount to 25% or even more, it becomes not only impractical but impossible to use the electrolytic method of separation.

Tin and lead as well as antimony and lead 40 form solid solutions and eutectic mixtures. Tin, antimony and lead form, beside solid solutions and ternary eutectics, intermetallic 45 compounds. The foregoing explains why lead cannot be separated from tin, antimony and their various alloys by physico-metallurgical means, such as liquation, fractional crystallization, centrifugal separation, etc.

50 The common methods of purification and

separation by chemico-metallurgical means, such as oxidation, sulphurization, etc., are also of no avail because tin and antimony are more reactive towards oxygen, etc., than lead is. I discovered, that vapors of anhydrous metallic chlorides existing in their highest state of oxidation such as stannic-chloride (SnCl<sub>4</sub>) or antimonio-chloride (SbCl<sub>5</sub>) conducted through a metal like molten tin, 55 antimony or their various alloys containing lead, zinc, cadmium and other constituents, will combine with said lead, zinc, etc., to form lead-chloride, zinc-chloride, etc. The anhydrous metallic chlorides in turn are either completely reduced to metal or to a 60 lower state of oxidation according to the equations.



70

The reactions appear to be nonreversible at any concentration.

The anhydrous metallic chlorides such as stannic and antimonio chlorides are liquids at ordinary temperature and their boiling 75 points are but a little above the boiling point of water. They are easily obtained from their components and in their anhydrous form, they are noncorrosive upon the ordinary materials of construction. In view of these, the process can be carried out in a very simple and cheap equipment. The latter may consist of an ordinary cast iron melting kettle to melt and hold the metal to be treated, said kettle being provided with 80 a tightfitting cover. Through said cover passes one or a plurality of pipes connected to a suitably heated container, said pipes extending into the molten metal. Said cover is also provided with one or a plurality of 85 outlets which are connected to a suitable condensing apparatus to condense and reclaim any such reagent which passed through the molten metal unaltered or which formed during the process and volatilizes 90 at the temperatures prevailing in said melting kettle. The anhydrous metallic-chloride is placed in the container and is heated to its boiling point. The vapors passing 95 through the metal will combine with the lead 100

or zinc, etc., if any present, such chlorides being lighter than the metal and remain on the surface of it from whence they can be removed, or they may volatilize in which case they are recovered by condensation as stated above.

As a specific example of my invention, 10,000 pounds of an alloy containing 92% tin, 6% lead and 2% antimony and heated 10 to 498°C. was treated as described with the vapors of 400 pounds of stannic chloride and obtained 9,760 pounds of an alloy containing 97.90% tin and 2.1% antimony, also 804 pounds of lead-chloride and recovered 15 26 pounds of unaltered anhydrous stannic chloride.

It is evident from the foregoing that various modifications and combinations of the process are possible which come under the 20 broader spirit of the invention. When a chloride is reduced to a lower form of oxidation from a higher form, nascent chlorine forms. It is this nascent chlorine which combines with the lead or zinc or other constituents and the behavior of this nascent chlorine is utterly different from the behavior of elemental chlorine. Elemental chlorine will react in an alloy of tin and lead with the tin primarily, while nascent chlorine reacts with the lead only. Stannic and 25 antimonio chlorides are convenient sources of nascent chlorine.

What I claim is:

1. The process of separating and recovering lead from tin or alloys of tin consisting in subjecting said tin or alloys of tin in the molten state to the action of vapors of anhydrous stannic chloride.
2. The process of purifying impure tin 40 and alloys of tin consisting in subjecting said tin and alloys of tin in the molten state to the action of vapors of anhydrous stannic chloride.

ALBERT HANAK.

45

50

55

60

65